

Feb. 16, 1926.

1,573,707

W. F. HOERLE

STEEL GOLF CLUB SHAFT

Filed Nov. 18, 1924

Fig. 1.



Fig. 2.



Fig. 3.



Fig. 4.



Fig. 5.



Fig. 6.



Fig. 7.



INVENTOR

William F. Hoerle

BY

R. S. BURGESS  
ATTORNEY

## UNITED STATES PATENT OFFICE.

WILLIAM FERDINAND HOERLE, OF TORRINGTON, CONNECTICUT, ASSIGNOR TO UNION HARDWARE COMPANY, OF TORRINGTON, CONNECTICUT, A CORPORATION OF CONNECTICUT.

## STEEL GOLF-CLUB SHAFT.

Application filed November 18, 1924. Serial No. 750,516.

To all whom it may concern:

Be it known that I, WILLIAM F. HOERLE, a citizen of the United States of America, residing at Torrington, county of Litchfield, 5 State of Connecticut, have invented a new and useful Steel Golf-Club Shaft, of which the following is a specification.

My invention relates to handles or shafts for golf clubs.

10 The ordinary wooden shaft is, of course, quite flexible and has desirable torsional characteristics which make the club lively, but it is very fragile, uncertain in quality and considerably affected by moisture. It 15 has heretofore been proposed to make such devices of steel. Some of these devices, however, have been very heavy and rigid and others very fragile. Shafts have been made of steel strips formed into tubes but these 20 are difficult to make uniformly and are likely to split open. So far as I know no one has heretofore been able to produce commercially an integral or seamless tubular golf club shaft sufficiently well balanced, 25 light and pliable to be useful and yet sufficiently strong to stand the severe stresses to which such a shaft is subjected.

The main object of my invention is to provide a light but strong, smooth and durable 30 metallic shaft which will look and act very much like a first-class wooden shaft and yet not have the objectionable characteristics of wood.

I have also sought to provide a shaft 35 capable of commercial production according to standard specifications and at a low cost.

I have found it possible to make a satisfactory shaft from an ordinary cylindrical 40 low carbon seamless steel tube by shaping or drawing it into taper form, then carbonizing the tapered tube and heat treating and finishing it.

Figure 1 is a side view of a golf club of 45 standard form having a shaft embodying my invention.

Fig. 2 is a side view of a tubular blank from which a shaft is made.

Fig. 3 is a side view of the finished shaft. 50 Figs. 4 and 5 are transverse sectional views of the shaft on an enlarged scale taken respectively at the upper and lower ends of the shaft.

Figs. 6 and 7 are enlarged detail sectional

views showing different ways of fastening 55 a shaft in a head.

The blank 7 is preferably of seamless tubing of low carbon steel having say from 10 to 20 points of carbon, that is from .1 to .2 of one per centum of carbon. The outside 60 diameter of the blank is preferably about  $\frac{5}{8}$  of an inch. The gauge of the metal is preferably from .015" to .018", although it may be lighter or heavier. About .016" is 65 quite desirable for a driver shaft.

This blank is rolled or swaged to the desired taper. For instance an ordinary golf club shaft would be something over 3 feet long and approximately  $\frac{5}{16}$  of an inch in diameter at the smallest point in the neck 70 8. The tapering process should preferably elongate the tube and draw it down so that there will be less metal in the cross-section in the smallest point than there is in the largest diameter of the tube and leave the 75 wall thicker in the neck than at the larger end. An elongation of ten per cent is usual. That is, from say 36" to 40". The torsibility of the tube gradually increases as the section is taken nearer the small end. This 80 also makes the tube more flexible in the neck. A satisfactory thickness of the wall at the neck would be .019", although it may be a little thicker or a little thinner than this.

After the tube has been worked to the desired shape and size, it is carbonized in a suitable manner, for instance in a gas fired tube or in a charcoal or coke furnace or electrically. This is done, preferably, at a 90 comparatively low temperature, say 1450° F. so as not to injure the steel. This carbonizing is continued until the carbon content of the steel is increased to a suitable amount for the purpose required, say from six tenths to one per centum. The carbon content can be increased even somewhat above one per cent by careful treatment but I do not consider it necessary to go above .75 to .80 and in some cases a tube with even less than .75 per centum of carbon can be 95 heat treated and hardened. The tube is then heat treated and drawn to the desired temper and then provided with a suitable non-corrosive finish. Such a shaft should weigh from about five to six ounces.

The length of course is a matter of accommodation to the individual. The weight will

necessarily vary with the length. The weight and stiffness of some clubs is of course less critical than others. For instance, a putter shaft does not need to be as flexible or torsible as a driver.

A low carbon steel tube is not only less expensive than a high carbon tube but it is much cheaper and easier to work without injury to the metal. The rolling or 10 swaging is preferably done cold and not only compacts the metal but draws out the fibre in the direction of the length of the shaft particularly in the smaller part so as to utilize the strength of the metal of 15 its maximum extent. The carbonizing and heat treating processes release the internal stresses developed by the prior working process and make the steel susceptible of hardening and tempering to a higher degree than would be possible with a low 20 carbon steel. Carbonizing of a low carbon steel when properly done produces a condition where there is more carbon in the metal near the surface than there is inside. 25 Consequently when hardened and tempered we have a hard exterior or skin and a softer interior and the tube is resilient and yet tougher and stronger than is possible to get in a tube made from a so called high 30 carbon steel.

The upper or handle end 9 of the tube may be left of uniform diameter if desired and provided with any suitable form of grip 10.

35 The shaft may be used with any style head. In Figure 1 I have shown a putter or iron provided with a socket 11. To fit such a socket I may provide the lower end of the shaft with a tapered enlargement 40 12 integral with the shaft and adapted to be fitted and held in the socket of the head in the same manner that a wooden shaft is held. It should be understood, of course, however, that the lower end may be inserted and held in any form of wooden head 45 in substantially the same manner that a wooden shaft is held.

In some cases it may be desirable to reinforce the tube adjacent the head by means 50 of a ferrule or plug such as 13 in Fig. 6. The curved end adjacent the entrance to the socket in the head 14 permits slight bending of the shaft and yet reinforces it at this point where the stress is very great.

In case the socket 15 of the head is larger 55 than the end of the shaft I may employ a filler ferrule 16. An inner plug 17 may be used to spread the end of the shaft in the socket and prevent the metal from buckling.

60 A pin 18 may be used to hold the parts together. The filler and plug both serve to reinforce the tube at this point.

Such a shaft not only has the requisite strength to resist crushing and bending but it has torsional and flexible characteristics closely resembling those of a wooden shaft of high grade. Since the shaft is drawn, rolled or swaged from a seamless tube, there are no joints liable to open when the club 70 is used and subjected to the severe strains of ordinary play. By this process it is possible to make shafts commercially in quantity production and with such standard characteristics as may be desired as to cost, 75 weight, flexibility and torsibility.

The method or process of forming the shaft is claimed in my application 41,229 filed July 2, 1925.

80 I claim:

1. A flexible, torsionable, seamless, thin-walled, tubular golf club shaft smaller in diameter at one end than at the other, formed of a low carbon steel tube mechanically worked so as to elongate it and reduce 85 the diameter at one end, carbonized to increase the carbon content at the surface to at least six tenths of one per cent of carbon, said shaft being heat treated, hardened and tempered.

2. A torsionable seamless tubular golf club shaft formed of low carbon steel rolled longitudinally, carbonized to increase carbon content at the surface, heat treated and tempered.

90 3. A torsionable seamless tubular golf club shaft formed of low carbon steel and having its fibre elongated longitudinally and carbonized, heat treated and tempered and containing approximately .75 per centum 100 of carbon.

4. A torsionable tapered tubular golf club shaft formed of low carbon seamless steel tubing about .016 thick, carbonized to contain from six tenths to one per centum of 105 carbon in the surface layer and weighing about five to six ounces.

WILLIAM FERDINAND HOERLE.